

[54] DI AND TRI (HYDROCARBYLAMMONIUM)  
TRITHIOCYANURATE AND LUBRICATING  
OIL COMPOSITIONS CONTAINING SAME

[75] Inventor: **John W. Nebzydoski**, Fishkill, N.Y.

[73] Assignee: **Texaco Inc.**, New York, N.Y.

[22] Filed: **Nov. 19, 1973**

[21] Appl. No.: **417,153**

[52] U.S. Cl. .... **252/33.6**, **252/47**, **260/248 CS**

[51] Int. Cl. .... **C10m 1/38**, **C10m 1/32**

[58] Field of Search..... **252/33.6**, **47**; **260/248 CS**

[56] **References Cited**

UNITED STATES PATENTS

2,223,130 11/1940 Prutton ..... **252/33.6**

2,676,150 4/1954 Loughran et al. .... **252/47**  
3,778,368 12/1973 Nakamura et al. .... **260/248 CS**

*Primary Examiner*—W. Cannon

*Attorney, Agent, or Firm*—T. H. Whaley; C. G. Ries

[57] **ABSTRACT**

Di- and tri- $C_8C_{24}$  hydrocarbyl ammonium trithiocyanurate and a lubricating oil composition containing said di- or tri- hydrocarbyl ammonium thithiocyanurate having improved load carrying properties.

**10 Claims, No Drawings**

DI AND TRI (HYDROCARBYLAMMONIUM)  
TRITHIOCYANURATE AND LUBRICATING OIL  
COMPOSITIONS CONTAINING SAME

## BACKGROUND OF THE INVENTION

## Field of the Invention

This invention relates to a novel hydrocarbylammonium trithiocyanurate produced by combining 2 to 3 moles of a C<sub>8</sub> to C<sub>24</sub> hydrocarbylamine with trithiocyanuric acid. These compounds can be described as the di- and trihydrocarbylamine salts of trithiocyanuric acid.

The di- and trihydrocarbylaminium trithiocyanurates are represented by the following formula:



in which R represents hydrogen or a hydrocarbyl radical having from 8 to 24 carbon atoms at least one R being a hydrocarbyl radical and n has a value from 0 to 1.

This invention also relates to a novel lubricating oil composition containing the above-described hydrocarbylaminium trithiocyanurate.

## SUMMARY OF THE INVENTION

In general, the di-and trihydrocarbylaminium trithiocyanurates are represented by the following formula:



in which R is hydrogen or a hydrocarbyl radical having from 6 to 24 carbon atoms at least one R being a hydrocarbyl radical and n has a value from 0 to 1. The so-defined hydrocarbylaminium trithiocyanurates result from the combination of from 2 to 3 moles of a hydrocarbylamine with trithiocyanuric acid. Hydrocarbylaminium trithiocyanurates formed from 1 mole of a hydrocarbylamine and a mole of trithiocyanuric acid are not suitable for the purpose to which the present invention is directed and are outside the scope of this invention.

A preferred class of compounds within the scope of this invention are the hydrocarbylaminium trithiocyanurates represented by the following formula:



in which R is a hydrocarbyl radical having from about 12 to about 22 carbon atoms.

Another preferred class of hydrocarbylaminium trithiocyanurates are represented by the formula:



15 in which R is a hydrocarbyl radical having from about 12 to about 22 carbon atoms. The hydrocarbyl radicals represented by R in all of the formulas above are monovalent hydrocarbyl or hydrocarbon radicals and include alkyl, aralkyl, aryl, alkaryl and cycloalkyl radicals having the prescribed carbon chain length.

A more preferred hydrocarbylaminium trithiocyanurate is that formed from tertiary alkyl primary amines wherein 2 or 3 moles of a tertiary alkyl primary amine has been reacted with trithiocyanuric acid.

20 The hydrocarbylaminium trithiocyanurates are conveniently prepared in a 2-step process beginning with cyanuric chloride. In the first step of this process, cyanuric chloride and thiourea are reacted in the presence of an inert solvent at a moderate temperature, generally the reflux temperature of the solvent to produce a solid reaction product. The solid product is filtered off and dissolved in an alkali solution, such as an aqueous potassium hydroxide solution, which is then acidified with a mineral acid, such as concentrated hydrochloric acid, to produce cyanuric acid, a pale yellow solid having a melting point of >300°C. The general procedure is given in the "Canadian Journal of Chemistry" 44 829 (1966). This reaction is illustrated by the following formula:

25

30

35

40

45

50

55

60

65

70

75

80

85

90

95

100

105

110

115

120

125

130

135

140

145

150

155

160

165

170

175

180

185

190

195

200

205

210

215

220

225

230

235

240

245

250

255

260

265

270

275

280

285

290

295

300

305

310

315

320

325

330

335

340

345

350

355

360

365

370

375

380

385

390

395

400

405

410

415

420

425

430

435

440

445

450

455

460

465

470

475

480

485

490

495

500

505

510

515

520

525

530

535

540

545

550

555

560

565

570

575

580

585

590

595

600

605

610

615

620

625

630

635

640

645

650

655

660

665

670

675

680

685

690

695

700

705

710

715

720

725

730

735

740

745

750

755

760

765

770

775

780

785

790

795

800

805

810

815

820

825

830

835

840

845

850

855

860

865

870

875

880

885

890

895

900

905

910

915

920

925

930

935

940

945

950

955

960

965

970

975

980

985

990

995

1000

1005

1010

1015

1020

1025

1030

1035

1040

1045

1050

1055

1060

1065

1070

1075

1080

1085

1090

1095

1100

1105

1110

1115

1120

1125

1130

1135

1140

1145

1150

1155

1160

1165

1170

1175

1180

1185

1190

1195

1200

1205

1210

1215

1220

1225

1230

1235

1240

1245

1250

1255

1260

1265

1270

1275

1280

1285

1290

1295

1300

1305

1310

1315

1320

1325

1330

1335

1340

1345

1350

1355

1360

1365

1370

1375

1380

1385

1390

1395

1400

1405

1410

1415

1420

1425

1430

1435

1440

1445

1450

1455

1460

1465

1470

1475

1480

1485

1490

1495

1500

1505

1510

1515

1520

1525

1530

1535

1540

1545

1550

1555

1560

1565

1570

1575

1580

1585

1590

1595

1600

1605

1610

1615

1620

1625

1630

1635

1640

1645

1650

1655

1660

1665

1670

1675

1680

1685

1690

1695

1700

1705

1710

1715

1720

1725

1730

1735

1740

1745

1750

1755

1760

1765

1770

1775

1780

1785

1790

1795

1800

1805

1810

1815

1820

1825

1830

1835

1840

1845

1850

1855

1860

1865

1870

1875

1880

1885

1890

1895

1900

1905

1910

1915

1920

1925

1930

1935

1940

1945

1950

1955

1960

1965

1970

1975

1980

1985

1990

1995

2000

2005

2010

2015

2020

2025

2030

2035

2040

2045

2050

2055

2060

2065

2070

2075

2080

2085

2090

2095

2100

2105

2110

2115

2120

2125

2130

2135

2140

2145

2150

2155

2160

2165

2170

2175

2180

2185

2190

2195

2200

2205

2210

2215

2220

2225

2230

2235

2240

2245

2250

2255

2260

2265

2270

2275

2280

2285

2290

2295

2300

2305

2310

2315

2320

2325

2330

2335

2340

2345

2350

2355

2360

2365

2370

2375

2380

2385

2390

2395

2400

2405

2410

2415

2420

2425

2430

2435

2440

2445

2450

2455

2460

2465

2470

2475

2480

2485

2490

2495

2500

2505

2510

2515

2520

2525

2530

2535

2540

2545

2550

2555

2560

2565

2570

2575

2580

2585

2590

2595

2600

2605

2610

2615

2620

2625

2630

2635

2640

2645

2650

2655

2660

2665

2670

2675

2680

2685

2690

2695

2700

2705

2710

2715

2720

2725

2730

2735

2740

2745

2750

2755

2760

2765

2770

2775

2780

2785

2790

2795

2800

2805

2810

2815

2820

2825

2830

2835

2840

2845

2850

2855

2860

2865

2870

2875

2880

2885

2890

2895

2900

2905

2910

2915

2920

2925

2930

2935

2940

2945

2950

2955

2960

2965

2970

2975

2980

2985

2990

2995

3000

3005

3010

3015

3020

3025

3030

3035

3040

3045

3050

3055

3060

3065

3070

3075

3080

3085

3090

3095

3100

3105

3110

3115

3120

3125

3130

3135

3140

3145

3150

3155

3160

3165

3170

3175

3180

3185

3190

3195

3200

3205

3210

3215

3220

3225

3230

3235

3240

3245

3250

3255

3260

3265

3270

3275

3280

3285

3290

3295

3300

3305

3310

3315

3320

3325

3330

3335

3340

3345

3350

3355

3360

3365

3370

3375

3380

3385

3390

3395

3400

3405

3410

3415

3420

3425

3430

3435

3440

3445

3450

3455

3460

3465

3470

3475

3480

3485

3490

3495

3500

3505

3510

3515

3520

3525

3530

3535

3540

3545

3550

3555

3560

3565

3570

3575

3580

3585

3590

3595

3600

3605

3610

3615

3620

3625

3630

3635

3640

3645

3650

3655

3660

3665

3670

3675

3680

3685

3690

3695

3700

3705

3710

3715

3720

3725

3730

3735

3740

3745

3750

3755

3760

3765

3770

3775

3780

3785

3790

3795

3800

3805

3810

3815

3820

3825

3830

3835

3840

3845

3850

3855

3860

3865

3870

3875

3880

3885

3890

3895

3900

3905

3910

3915

3920

3925

3930

3935

3940

3945

3950

3955

3960

3965

3970

3975

3980

3985

3990

3995

4000

4005

4010

4015

4020

4025

4030

4035

4040

4045

4050

4055

4060

4065

4070

4075

4080

4085

4090

4095

4100

4105

4110

4115

4120

4125

4130

4135

4140

4145

4150

4155

4160

4165

4170

4175

4180

4185

4190

4195

4200

4205

4210

4215

4220

4225

4230

4235

4240

4245

4250

4255

4260

4265

4270

4275

4280

4285

4290

4295

4300

4305

4310

4315

4320

4325

4330

4335

4340

4345

4350

4355

4360

4365

4370

4375

4380

4385

4390

4395

4400

4405

4410

4415

4420

4425

4430

4435

4440

4445

4450

4455

4460

4465

4470

4475

4480

4485

4490

4495

4500

4505

4510

4515

4520

4525

4530

4535

4540

4545

4550

4555

4560

4565

4570

4575

4580

4585

4590

4595

4600

4605

4610

4615

4620

4625

4630

4635

4640

4645

4650

4655

4660

4665

4670

4675

4680

4685

4690

4695

4700

4705

4710

4715

4720

4725

4730

4735

4740

4745

4750

4755

4760

4765

4770

4775

4780

4785

4790

4795

4800

4805

4810

4815

4820

4825

4830

4835

4840

4845

4850

4855

4860

4865

4870

4875

4880

4885

4890

4895

4900

4905

4910

4915

4920

4925

4930

4935

4940

4945

4950

4955

4960

4965

4970

4975

4980

4985

4990

4995

5000

5005

5010

5015

5020

5025

5030

5035

5040

5045

5050

5055

5060

5065

5070

5075

5080

5085

5090

5095

5100

5105

5110

5115

5120

5125

5130

5135

5140

5145

5150

5155

5160

5165

5170

5175

5180

5185

5190

5195

5200

5205

5210

5215

5220

5225

5230

5235

5

In the second step of the process, trithiocyanuric acid and 2 to 3 moles of a hydrocarbylamine per mole of trithiocyanuric acid are reacted as illustrated by the following formula:



where  $n$  equals 0 or 1.

The reactants are heated at an elevated temperature ranging up to 220° to 260°F. with adequate stirring. On completion of this reaction, the product is diluted with methanol or ethanol, filtered, and the salt recovered from the hydrocarbon solvent generally in the form of a yellow oil.

As indicated above, the hydrocarbyl ammonium tri-thiocyanurate employed in this invention will contain 2 to 3 moieties of the hydrocarbylamine per mole of the trithiocyanuric acid moiety. The hydrocarbylamine is represented by the formula  $RNH_2$  in which R represents a hydrocarbyl radical having from 8 to 24 carbon atoms. Preferred amines are those in which R is a hydrocarbyl radical having from about 12 to 22 carbon atoms. The hydrocarbyl radical can be any monovalent organic radical, such as an alkyl, aryl, cycloalkyl, alkaryl or aralkyl hydrocarbon radical of the indicated carbon chain length. The alkyl radical can be a straight-chain or branched-chain hydrocarbon radical although it is preferred to employ amines in which the hydrocarbyl radical is a tertiary alkyl saturated hydrocarbon radical.

The following examples illustrate the preparation of typical hydrocarbyl ammonium trithiocyanurates according to this invention.

## DESCRIPTION OF THE PREFERRED EMBODIMENTS

### EXAMPLE I

### Tri (t-C<sub>18</sub>to C<sub>22</sub>primary ammonium) trithiocyanurate

18.45 parts of cyanuric chloride, 22.8 parts of thiourea and 400 parts of acetone were refluxed for 2 hours. The solid product was filtered off and dissolved in 170 parts of potassium hydroxide solution (115 grams  $H_2O$ /20 grams KOH). This mixture was acidified to a pH of 1 with concentrated hydrochloric acid yielding as product a pale yellow solid having a melting point greater than 300°C. The infrared spectrum of this sample was taken and found to be identical to that of an authentic sample.

5.31 parts of trithiocyanuric acid and 28.4 parts of t-C<sub>18</sub> to C<sub>22</sub> alkyl primary amine were heated for about 2 hours at 220°F. with stirring. The reaction mixture was cooled, diluted with 50 parts of methanol, filtered and concentrated yielding the product as a yellow oil. This product conformed to the following formula:



in which R represents a t-C<sub>18</sub> to C<sub>24</sub> aliphatic hydrocarbon radical. This salt had a nitrogen content of 7.6 percent (calc. 7.6) and a sulfur content of 8.4 percent (calc. 8.6).

### EXAMPLE II

### Tri(t-C<sub>11</sub>-C<sub>14</sub> alkyl primary ammonium) trithiocyanurate

25 2.95 parts of tri thiocyanuric acid and 9.55 parts of t-C<sub>11</sub>-C<sub>14</sub> primary alkylamine were heated for about 2 hours at about 250°F. with stirring. The reaction product was cooled, diluted with ethanol, filtered and concentrated yielding 11.9 parts of tri(t-C<sub>11</sub>-C<sub>14</sub> alkyl primary ammonium) trithiocyanurate as a yellow oil. This product has a nitrogen content of 11.7 percent (calc. 12.0).

### EXAMPLE III

<sup>35</sup> Di-(t-C<sub>18</sub>-C<sub>22</sub> alkyl primary ammonium) trithiocyanurate

5.31 parts of trithiocyanuric acid and 18.9 parts of t-C<sub>18</sub>-C<sub>22</sub> alkyl primary amine were reacted as in Example I above to form di(t-C<sub>18</sub>-C<sub>22</sub> alkyl primary ammonium) trithiocyanurate having a nitrogen content of 9.6 (calc. 8.7) and a sulfur content of 11.5 (calc. 11.9).

Many other oil-soluble di- and trihydrocarbylammonium trithiocyanurates can be prepared within the scope of this invention following the above procedure which are useful for enhancing the load-carrying properties of a lubricating oil composition. Additional examples of these compounds include di- and tri-(octadecylammonium) trithiocyanurate, di- and tri-(trioctadecyl-ammonium) trithiocyanurate, di- and tri-(dioctadecyl ammonium) trithiocyanurate, di- and tri-(di-t-C<sub>11</sub>-C<sub>14</sub> alkyl ammonium) trithiocyanurate, di- and tri-(tri-t-C<sub>11</sub>-C<sub>14</sub> alkylammonium) trithiocyanurate, di- and tri-(hexadecylammonium) trithiocyanurate, di- and tri-(dectylammonium) trithiocyanurate, di- and tri-(eicosylammonium) trithiocyanurate, di- and tri-(dodecylammonium) trithiocyanurate, and di- and tri-(octylammonium) trithiocyanurate.

The di- and tri-(hydro carbylammmonium) trithiocyanurate 60 of this invention are valuable for enhancing the load-carrying properties of lubricating oils. In general, the prescribed compounds can be employed in both mineral and synthetic lubricating oil compositions usually at a concentration ranging from about 0.001 to 65 about 0.5 weight percent with the preferred concentration being from about 0.01 to 0.3 percent. A suitable mineral lubricating oil base will have an SUS viscosity at 100°F. ranging from about 50 to 1,000 with the pre-

ferred viscosity range being from 70 to 300 SUS at 100°F.

The prescribed additive compounds of this invention are particularly efficacious in synthetic ester base lubricating oil compositions and were employed in a typical fully formulated synthetic ester base lubricating oil which was tested for its load-carrying properties as well as for its oxidation-corrosion resistance.

The base fluid component of this type lubricant is an ester-base fluid prepared from pentaerythritol or trimethylolpropane and a mixture of hydrocarbyl monocarboxylic acids. Polypentaerythritols, such as dipentaerythritol, tripentaerythritol and tetra-pentaerythritol can also be employed in the reaction to prepare the base oil.

The hydrocarbon monocarboxylic acids which are used to form the ester-base fluid include the straight-chain and branched-chain aliphatic acids, cycloaliphatic acids and aromatic acids as well as mixtures of these acids. The acids employed have from about 2 to 18 carbon atoms per molecule, and preferably from about 5 to 10 carbon atoms. Examples of suitable specific acids are acetic, propionic, butyric, valeric, isovaleric, caproic, decanoic, cyclohexanoic, benzoic acid, phenylacetic, tertiary-butylacetic acid and 2-ethylhexanoic acid.

In general, the acids are reacted in proportions leading to a completely esterified pentaerythritol or trimethylolpropane with the preferred ester bases being the pentaerythritol tetraesters. Examples of such commercially available tetraesters include pentaerythritol tetracaproate, which is prepared from purified pentaerythritol and crude caproic acid containing other C<sub>5-10</sub> monobasic acids. Another suitable tetraester is prepared from a technical grade pentaerythritol and a mixture of acids comprising 38 percent valeric, 13 percent 2-methyl pentanoic, 32 percent octanoic and 17 percent pelargonic acids. Another effective ester is the triester of trimethylolpropane in which the trimethylolpropane is esterified with a monobasic acid mixture consisting of 2 percent valeric, 9 percent caproic, 13 percent heptanoic, 7 percent octanoic, 3 percent caprylic, 65 percent pelargonic and 1 percent capric acids. Trimethylolpropane triheptanoate is also a suitable ester base.

The ester base comprises the major portion of the fully formulated synthetic ester base lubricating oil composition. In general, this ester base fluid is present in concentrations from about 90 to 98 percent of the composition.

In addition to the essential di- or tri- (hydrocarbylaminium) trithiocyanurate component of the lubricating oil composition, synthetic ester base lubricants will generally contain additional additives to impart oxidation and corrosion resistance, metal deactivators and the like in order to provide a superior lubricant composition.

A valuable oxidation and corrosion inhibitor is an alkyl or alkaryl phenyl naphthylamine represented by the formula:



in which R is an alkyl or alkaryl radical having from about 3 to 12 carbon atoms. This radical can be a straight or branched chain alkyl radical with the ter-

tiary alkyl structure being preferred or it can be an alkylaryl radical. The naphthylamine can be either an alpha or beta naphthylamine. Specific effective compounds of this class include N-(p-t-octylphenyl)- $\alpha$ -naphthylamine, N-(4-cumylphenyl)-6-cumyl- $\beta$ -naphthylamine, N-(p-t-octylphenyl)- $\beta$ -naphthylamine and the corresponding p-t-dodecylphenyl, p-t-butylphenyl, and p-dodecylphenyl- $\alpha$  and - $\beta$ -naphthylamines. The preferred naphthylamines are those in which R is a tertiary alkyl radical having from 6 to 10 carbon atoms with the preferred concentration of this component being from about 0.5 to 2.5 percent.

Another valuable oxidation inhibitor of the ester base lubricating oil composition is a dialkyl diphenylamine. 15 These compounds are represented by the formula:



in which the R is an alkyl radical having from about 3 to 12 carbon atoms. Suitable alkylamines include dioctyldiphenylamine, didecyldiphenylamine and similar compounds. The preferred class of dialkyl diphenylamines are those in which R is an alkyl radical having from 8 to 10 carbon atoms. Dooctyldiphenylamine is the preferred compound and the effective concentration is from 0.5 to 2.0 percent.

Another valuable component of an ester base lubricating oil composition is a hydrocarbylphosphate ester, more specifically a trihydrocarbyl phosphate having the formula (RO)<sub>3</sub>PO in which R is a hydrocarbyl radical, i.e., an alkyl, aryl, alkaryl, cycloalkyl or aralkyl radical or mixture thereof having from 2 to 12 carbon atoms and preferably from 4 to 8 carbon atoms. Effective specific compounds include tricresylphosphate, cresyl diphenyl-phosphate, triphenylphosphate, tributylphosphate, tri(2-ethylhexyl)-phosphate and tricyclohexyl phosphate. These compounds are generally effective at a concentration ranging from about 0.5 to 5 weight percent of the lubricant composition.

An optional component of the lubricant is a metal deactivator, which is commonly employed in an ester base lubricating oil composition. An effective metal deactivator is a polyhydroxy-substituted anthraquinone inhibitor represented by the formula:



in which X, Y and Z each represent hydrogen or a hydroxyl group and at least one of these is a hydroxyl group. Examples of effective polyhydroxy-substituted anthraquinones include 1,4-dihydroxyanthraquinone, 1,5-dihydroxyanthraquinone, 1,2,4-trihydroxyanthraquinone and 1,2,5,8-tetrahydroxyanthraquinone. In general, this component is employed in a concentration ranging from about 0.04 to 2.0 weight percent of the lubricating oil composition with the preferred concentration being from 0.05 to 0.25 weight percent.

The load carrying properties of lubricants containing trithiocyanurates was determined by preparing oil compositions and subjecting them to load-carrying tests in

the Ryder Gear Test. The lubricating oil compositions were also tested for their oxidation and corrosion resistance in the 425°F/48 Hr. Oxidation and Corrosion Test which was conducted in accordance with Standard No. 791a (issued Dec. 31, 1961) except for modifications to conform to Pratt and Whitney 521C Specifications. The bath temperature is maintained at 425°F.  $\pm$  1°F. instead of at 250°F. and the test is conducted for a period of 48 hours instead of 168 hours as specified in the original test.

The ester base oil employed in preparing Base Fluids A and B below comprised pentaerythritol containing a minor amount of dipentaerythritol esterified with mixtures of fatty acids. This ester base (Hercules L-39) consisted of a technical grade pentaerythritol ester made from a mixture of carboxylic acids consisting of (mole percent).

|                           |            |
|---------------------------|------------|
| <i>i</i> - C <sub>5</sub> | $\pm 2\%$  |
| <i>i</i> - C <sub>5</sub> | 22 $\pm$ 5 |
| <i>n</i> - C <sub>6</sub> | 21 $\pm$ 5 |
| <i>n</i> - C <sub>7</sub> | 27 $\pm$ 5 |
| <i>n</i> - C <sub>8</sub> | 7 $\pm$ 3  |
| <i>n</i> - C <sub>9</sub> | 18 $\pm$ 3 |

This ester base oil had the following physical properties:

|                         |      |
|-------------------------|------|
| Viscosity, cs at 210°F. | 5.01 |
| Viscosity, cs at 100°F. | 25.6 |
| Viscosity, cs at -40°F. | 7005 |
| Viscosity Index         | 140  |
| Flash, °F.              | 515  |

Base Fluid A consisted of 95.4 weight percent of the foregoing ester base plus 1.0 weight percent dioctyldiphenylamine, 1.5 wt. percent N-(4-tert.octylphenyl)- $\alpha$ -naphthylamine 2.0 wt. percent tricresylphosphate, and 0.1 wt. percent of quinizarin. This Base Fluid has an average Ryder Gear Test Failure Load of about 2,650 ppi.

Base Fluid B was similar to Base Fluid A but contained N-(4-cumylphenyl)-6-cumyl-2-naphthylamine in place of the N-(4-tert. octylphenyl)- $\alpha$ -naphthylamine. This Base Fluid has an average Ryder Gear Test Failure Load of about 2,650 ppi.

Base Fluid C is a reference oil used in the U.S. Navy's XAS-2354 specification (Hercolube A) as a comparison oil for evaluating high load oils. According to the U.S. Navy specifications, a high gear load oil passes this test if it exhibits a load carrying capacity of 144 percent (two runs) or 135 percent (six run average) over the reference oil.

The results of the Ryder Gear Load Carrying Test and the Oxidation-Corrosion Test are set forth in the table below:

The foregoing tests demonstrate the outstanding performance of the novel di- and tri-(hydrocarbylammonium) tri-thiocyanurate for increasing the load-carrying properties of a lubricating oil composition both in the Ryder Gear Load Test and according to the U.S. Navy's load-carrying test. The lubricants have also been shown to provide formulated blends which possess good Oxidation-Corrosion properties.

We claim:

1. A lubricant composition comprising a major portion of base oil having lubricating properties containing from about 0.001 to 0.5 wt. percent of a hydrocarbyl-ammonium trithiocyanurate represented by the formula:



in which R is hydrogen or a hydrocarbyl radical having from about 8 to 24 carbon atoms at least one R being a hydrocarbyl radical and n has a value from 0 to 1.

2. A lubricating oil composition according to claim 1 in which said hydrocarbyl radical has from 12 to 22 carbon atoms.

3. A lubricating oil composition according to claim 1 in which said hydrocarbyl radical is a tertiary alkyl hydrocarbon radical.

4. A lubricating oil composition according to claim 1 in which said hydrocarbyl ammonium trithiocyanurate is tri(t-C<sub>18</sub>-C<sub>22</sub> alkyl primary ammonium) trithiocyanurate.

5. A lubricating oil composition according to claim 1 in which said hydrocarbyl ammonium trithiocyanurate is tri(t-C<sub>11</sub>-C<sub>14</sub> alkyl primary ammonium, trithiocyanurate).

6. A lubricating oil composition according to claim 1 in which said hydrocarbyl ammonium trithiocyanurate is di(t-C<sub>18</sub>-C<sub>22</sub> alkyl primary ammonium, trithiocyanurate).

7. A lubricating oil composition according to claim 1 in which said hydrocarbyl ammonium trithiocyanurate is di(t-C<sub>11</sub>-C<sub>14</sub> alkyl primary ammonium) trithiocyanurate.

TABLE I

## EVALUATION OF DI- AND TRI-(HYDROCARBYLAMMONIUM) TRITHIOCYANURATES

| Run | Base Fluid   | Additive & Conc. Wt. % | RYDER GEAR TEST FAILURE LOAD |                          | 425°F/48 Hr. PWA-521C OXID. CORR TEST WT. $\Delta$ , mg/cm <sup>2</sup> |     |          |
|-----|--------------|------------------------|------------------------------|--------------------------|-------------------------------------------------------------------------|-----|----------|
|     |              |                        | ppi                          | % Herc. A <sup>(1)</sup> | Cu.                                                                     | Mg. | TAN Inc. |
| 1   | Base Fluid B | Example I 0.15         | 3185                         | 147                      | —                                                                       | —   | 23.0     |
| 2   | Base Fluid B | Example III 0.15       | 3015                         | 166                      | -0.29                                                                   | 0.0 | 0.74     |
| 3   | Base Fluid B | Example II 0.15        | 3460                         | 144                      | +0.21                                                                   | 0.0 | 1.11     |
| 4   | Base Fluid A | Example I 0.30         | 3850                         | 184                      | —                                                                       | —   | 28.5     |

<sup>(1)</sup> Relative rating in percent obtained by running the U.S. Navy reference oil "Base Fluid C" on the front side of the gear set and the test oil on the back side of the same gear set.

8. A lubricating oil composition according to claim 1 in which said base oil is a mineral oil.

9. A lubricating oil composition according to claim 1 in which said base oil is a synthetic ester base oil.

10. A lubricating oil composition according to claim 1 containing from about 0.5 to 2.5 percent of an alkary-

lphenyl- $\alpha$ -or $\beta$ naphthylamine, from about 0.5 to 2.0 percent of a dioctyldiphenylamine, from about 0.5 to 5 percent of a trihydrocarbyl phosphate and from about 0.05 to 0.25 percent of a polyhydroxyanthraquinone.

\* \* \* \* \*